

## UNITED STATES PATENT OFFICE

GUSTAVE R. ESPING, OF CLEVELAND, OHIO

## LUBRICATING COMPOUND FOR INSULATED ELECTRIC WIRES

No Drawing.

Application filed August 28, 1926. Serial No. 132,325.

This invention relates to a compound for application to insulated electric wires preparatory to pulling them through pipes or conduits commonly used for housing the wires 5 in the electric wiring of buildings and other structures, and to the method of producing such a compound.

It is well known that, in such electrical installations as above referred to, it is necessary to pull or draw insulated wires through 10 conduit systems which frequently involve very long and tortuous and more or less restricted passages, and unless the wires are lubricated in some way this work is extremely 15 difficult and is liable to result in injury to the insulation. This fact is more evident when it is remembered that the ordinary insulation on electric wires is more or less sticky, especially when subjected to the strain of the 20 pull necessary to draw such wires through the conduits or when exposed to heat even in a minor degree. Heretofore powdered soap-stone, ordinary soft soap or oil soap, oil and grease have often been used as lubricants for 25 this purpose, but such substances invariably react with marked deteriorating effects upon the insulation of the wires, and some of these substances have a tendency to coagulate in the conduit making it almost impossible, if 30 not quite so, to withdraw the wires from the conduits, which is often necessary in electric work, sometimes years after the original installation.

The object of my invention is to provide a 35 highly efficient compound for the purpose above set forth that has no ill effects upon the insulation and from which—after the compound has served its purpose—the moisture present therein evaporates, leaving only a 40 light powdery substance which presents no difficulties to, but rather enhances, the withdrawal of the wires from the conduits when such becomes necessary.

The compound has a saponaceous base. A 45 soap which I have found suitable for this

purpose contains the following ingredients in approximately the proportions named:

|                    | Per cent |
|--------------------|----------|
| Moisture           | 91       |
| Silica             | .96      |
| Oil of cotton seed | 2.20     |
| Potassium hydroxid | 5.84     |

With this base is compounded other substances as follows:

Five pounds of soap of the above general character is cut up and dissolved in eight quarts of water. This is heated to a temperature of from 160 to 180 degrees F. One-half pound of suet and one-half pound of slippery elm bark is placed in approximately six quarts of water and is boiled until they form a thick gruel-like substance to which sufficient water is added when necessary to bring the completed gruel-like substance up to a 65 quantity of five quarts. This gruel-like substance is added to the above eight quarts of soapy solution and is stirred in the presence of heat until the two are thoroughly mixed. The mixture is then removed from the influence of the heat and is placed in a suitable mixing machine and agitated until it becomes a foamy substance. The machine is then stopped and the mixture allowed to settle from three to five minutes. Next, cool water 70 is injected into the cooling jacket of the mixing machine around the mixing pot, and at the same time the mixture is stirred slowly, allowing it to take up and hold sufficient air to inflate the bulk of the compound to approximately four times its original size, and increase its foamy characteristics.

The compound is then cooled gradually to a temperature of approximately 60 degrees F. and placed in suitable containers—preferably paraffin coated wooden containers—having small drain openings at their bottom and permitted to stand in the same temperature for about ten days, which permits any free moisture to drain from the compound.

Following this, the mixture is placed in suitable receptacles, preferably paraffin coated, and sealed and is now ready for shipment or storage.

6 The completed preparation is a foamy, aerated substance having quick drying properties when exposed to the air for any appreciable length of time, and by reason of its qualities is peculiarly suited for use as a lubricant for insulated electric wires when pulling or drawing them through conduits.

10 Having thus described my invention, what I claim is:

15 1. The method of producing a lubricating compound for insulated electric conductors which consists in dissolving five pounds of a potash soap made from cottonseed oil in eight quarts of water, heating this solution to a temperature of from 160° to 180° F., placing 20 one-half pound suet and one-half pound of slippery elm bark in approximately six quarts of water and boiling the same until it forms a thick gruel-like substance, adding sufficient water to bring the complete 25 quantity of gruel-like substance up to five quarts, mixing the gruel-like substance and soap solution and stirring the same in the presence of heat until thoroughly mixed, removing the compound from the influence 30 of the heat and thoroughly agitating it until it has the consistency of a thick foam, next allowing the substance to stand for from two to five minutes, then cooling and stirring the compound slowly allowing it to take up and 35 hold a sufficient quantity of air to increase the bulk of the compound to approximately four times its original volume, allowing the compound to cool gradually to a temperature of about 60° F., and next placing the compound in containers and permitting it to stand subjected to a constant temperature for about ten days so as to allow any free 40 moisture to drain from the compound.

45 2. A lubricating compound for insulated wires comprising a potash soap, suet, slippery elm bark, and water in the approximate proportions by weight of soap five parts, suet one-half part, slippery elm bark one-half part and water twenty-six parts.

50 3. A lubricating compound for insulated wires comprising a potash soap made from cottonseed oil and including a small percentage of silica, suet, slippery elm bark and water in approximately the following proportions, soap five parts, suet one-half part, slippery elm bark one-half part and water twenty-six parts, said compound having sufficient air incorporated therewith to have the consistency of a foam.

55 60 In testimony whereof, I hereunto affix my signature.

GUSTAVE R. ESPING.